

## UNITED STATES PATENT OFFICE

VALENTIN DIETZ, OF FRANKFORT-ON-THE-MAIN, GERMANY, ASSIGNOR TO THE AMERICAN MULTIGRAPH COMPANY, OF CLEVELAND, OHIO, A CORPORATION OF OHIO

DRY-OFFSET-PRINTING PROCESS

REISSUED

No Drawing. Application filed June 18, 1928, Serial No. 293,779, and in Germany January 20, 1927.

My invention relates to an improved dry-offset printing process. It has been suggested heretofore to print by means of flat printing members without using a sponging liquid, but as far as my knowledge goes, this problem has not been solved in a satisfactory manner.

All attempts that have been made heretofore to substitute for the sponging or wiping water a means, such as the addition of acids or metallic salts to the preparing liquid, have proved a failure since, as soon as moistening is dispensed with, the printing member will at once take up and hold the printing ink outside of the figures to be typed so that accurate printing is impossible.

It has also been proposed heretofore, to mix so-called tone-protecting metallic salts or acids with the printing ink instead of the preparing liquid. All these prior suggestions, however, failed to be reliable substitutes for the old moistening operation the more so since they involve the disadvantage of injuriously affecting the prints and damaging the metal, so that the efficiency and life of the printing member will be considerably reduced thereby.

I have found, after much study and research, that absolutely tone-free prints or copies can be obtained by means of flat printing members if, in the case of employing aluminium as a printing metal, both the preparing liquid and the printing ink are mixed with the metallic nitrates or sulfates such as aluminium nitrate or sulphate. The nitrates of nickel, iron and copper can also be used. These salts do not injuriously affect the print nor the aluminium, and I have found that the said salts have a tone-protecting effect and at the same time act to improve the quality of the print, in contradistinction to the means hitherto employed or suggested, so that a great many more copies can be taken than hitherto possible in the wet-offset printing process.

Moreover, the use of metallic nitrates or sulfates, according to my invention, considerably simplifies the troublesome and precarious reprinting process as hitherto practised and affords a more reliable base to the latter.

When an aluminium plate is directly written upon or covered with drawings or the script-

ural characters are copied thereon by means of a suitable reprinting ink, it will be sufficient to moisten the plate inclusive of the scriptural characters with an aqueous solution of a metallic nitrate or sulfate and to apply thereto a printing ink which is likewise mixed with a metallic nitrate or a sulfate. The printing characters will be improved or enriched thereby and absorb the ink readily, whereas all other parts of the printing plate repel the ink thoroughly and remain absolutely tone-free. Any usual fatty ink or fatty pencil may be employed for writing the scriptural characters. In case of type-writing a black ink-ribbon of conventional nature will do, but particularly a ribbon cut from or consisting of ordinary carbon paper will give the best results. A carbon paper ribbon is inexpensive and has the further advantage of producing more precise, sharp and well-defined copies.

The steps of the process are as follows:

1. Ink image is located on an ordinary planographic metal plate by any suitable process, such as drawing directly on the plate with a lithographic crayon, transferring a design previously prepared on transfer paper, or by any other methods well known in photolithography for locating an image on a plate.

2. The plate is treated by covering the surface with a solution prepared in accordance with the present application. This solution is prepared by dissolving about 5% of metallic nitrates or sulphates or both in any kind of suitable liquid such as water.

3. The plate is now prepared for printing by rubbing the printing surface with said solution in order to condition it for the ink. This conditioning results from the solution leaving a film of crystals or particles of the metallic nitrates or sulphates on the fat-free surfaces of the plate, which film will subsequently prevent the adherence of the printing ink to the plate except on the previously prepared image. The solution will at the same time clean the surface of all foreign matter such as ink spots or dirt. The plate is then allowed to become perfectly dry and needs no further dampening for printing.

3a. A special ink has been prepared before-

- hand for applying on the plate. This ink is composed of any known common off-set ink containing for instance linseed oil and lamp-black or other coloring matter together with 5 to 8% of metallic nitrate or sulphate, or both, intimately mixed with the other ingredients. In the case of an aluminum plate, aluminum nitrate or aluminum sulphate would be used.
- 10 4. The plate needs no dampening and the special ink is now applied directly on the dried printing surface which does not retain ink on non-image areas which have a dry protective coating due to the treatment described.
- 15 5. The plate is now ready for printing and any number of copies can be made from the plate on which the ink is renewed by repeated applications. The supply of crystals 20 or particles in the non-image areas is replenished from the metallic nitrate or sulphate salts contained in the ink.
- 25 Apparently the metallic nitrate or sulphate solution applied to the plate leaves a deposit of fine particles or crystals of the metallic nitrate or sulphate on the plate, which particles adhere to the plate (assuming the latter is a fat-free substance) due to the natural adhesive quality of these particles 30 or crystals when applied to non-greasy substances. So far as I know, there is no actual chemical action on the plate. Since the printing ink contains a percentage of the metallic nitrates or sulphates, and since these 35 ingredients have no affinity for the ink, and are not chemically combined therein but mechanically mixed with the ink, the particles of metallic nitrates or sulphates in the ink replenish the supply of particles on the plate, 40 each time the roller bearing the ink is applied to the plate. Naturally, where the image appears on the plate (formed by fatty ink or pencil or by generally known photographic steps, or any known equivalent of the above), 45 the image bearing parts of the plate will not readily take up any of the particles of the metallic nitrates or sulphates from the ink, because such fatty ink image or equivalent naturally repels these particles.
- 50 5. It will be understood that I have mentioned an aluminum plate in the above disclosure by way of example only, and that the invention is applicable to substances other than aluminum which are suitable for use as 55 printing plates. I believe these materials include only those which are fat-free.
- 60 It will be evident that my invention, while still being adhered to in its main essentials, may be varied and adapted in many ways, according to requirements desired or most suitable under different circumstances.
- I claim:
1. A printing process, comprising the following steps, first, preparing a printing plate 65 with an image to be printed, and with a sub-

stance carrying a material selected from the group containing metallic nitrates and metallic sulphates, and then printing from such plate with an ink carrying a material selected from said group.

2. A printing process consisting in providing a text directly on a plate by means of a fatty ink and then treating said plate with a solution of a material selected from the group consisting of metallic nitrates and metallic sulphates and finally applying a fatty ink containing material selected from said group.

3. A printing process in which a printing plate is first provided with a text by means of a fatty ink, second, treating a plate with a solution of a material selected from a group containing metallic nitrates and metallic sulphates and printing from said plate with an ink which contains material from said group.

4. A printing process consisting in providing a text directly on a plate by means of a fatty ink and then treating said plate with a solution of a metallic nitrate and printing from said plate with an ink containing a metallic nitrate.

In testimony whereof I affix my signature.

VALENTIN DIETZ.

70

75

80

85

90

95

100

105

110

115

120

125

130